

# United States Patent [19]

Melzer et al.

[11]

4,155,764

[45]

May 22, 1979

[54] **PHOTOGRAPHIC COLOR DEVELOPER COMPOSITION**

[75] Inventors: **Arnfried Melzer, Cologne; Erwin Schön, Leverkusen, both of Fed. Rep. of Germany**

[73] Assignee: **AGFA-Gevaert, A.G., Leverkusen, Fed. Rep. of Germany**

[21] Appl. No.: **797,811**

[22] Filed: **May 17, 1977**

[30] **Foreign Application Priority Data**

May 21, 1976 [DE] Fed. Rep. of Germany ..... 2622950

[51] Int. Cl.<sup>2</sup> ..... **G03C 5/30**

[52] U.S. Cl. ..... **96/66.4; 96/56; 96/59**

[58] Field of Search ..... **96/66 R, 66.4, 56**

[56]

**References Cited**

**U.S. PATENT DOCUMENTS**

|           |         |                         |         |
|-----------|---------|-------------------------|---------|
| 2,936,308 | 5/1960  | Hodge .....             | 96/66.4 |
| 3,068,100 | 12/1962 | Dersch .....            | 96/66.4 |
| 3,582,333 | 6/1971  | Yost et al. .....       | 96/56   |
| 3,664,835 | 5/1972  | Youngquist .....        | 96/66 R |
| 3,700,442 | 10/1972 | Gabrielson et al. ..... | 96/66.4 |
| 3,846,129 | 11/1974 | Kuh .....               | 96/66 R |

**FOREIGN PATENT DOCUMENTS**

9537 of 1906 United Kingdom ..... 96/66.4

*Primary Examiner*—Mary F. Kelley

[57]

**ABSTRACT**

A photographic color developer composition containing a color developer compound and an antioxidant wherein it contains a water-soluble enolizable  $\alpha$ -aminocarbonyl compound as antioxidant is provided. Resistance to atmospheric oxygen of photographic color developer baths is improved.

**3 Claims, No Drawings**

PHOTOGRAPHIC COLOR DEVELOPER  
COMPOSITION

This invention relates to an aqueous alkaline colour developer composition containing novel antioxidants.

Hydroxylamine is one of the most common antioxidants in practice. It is known that hydroxylamine decomposes slowly under the influence of atmospheric oxygen and that this decomposition can be accelerated by certain other standard additives, for example heavy metal ions. Additives such as these greatly impair the stability of colour developer baths containing hydroxylamine. It has also been found that hydroxylamine not only acts as an antioxidant, but also apparently influences the results of development under certain conditions. For example, it has been found in reversal processing that the colour densities obtained during reversal development depend from the concentration of hydroxylamine.

It is obvious that, where the developer baths are used over fairly long periods, this does not lead to reproducible results, particularly when processing is carried out at elevated temperatures, especially since the concentration of the hydroxylamine can change quickly as a result of decomposition.

U.S. Pat. No. 3,615,503 describes the use of certain  $\alpha$ -hydroxy keto compounds as antioxidants for colour developer compositions which are said to be superior to hydroxylamine in preventing oxidation. Although a certain improvement in the stability of the colour developer compositions is obtained with some of these  $\alpha$ -hydroxy keto compounds, there is still a need to find other antioxidants with which the stability of colour developer compositions can be further improved.

The object of the present invention is to provide new antioxidants for aqueous alkaline colour developer compositions which show a reduced tendency towards decomposition or which influence the results of development to a lesser extent than hydroxylamine and which are superior to conventional antioxidants in their anti-oxidation effect.

The present invention provides a colour developer composition which contains a colour developer compound and an antioxidant, distinguished by the fact that it contains an enolisable  $\alpha$ -aminocarbonyl compound as the antioxidant. The antioxidants according to the invention contain groups capable of tautomerism as follows:



Accordingly, in the carbonyl form they contain, on the carbon atom between the nitrogen atom and the carbonyl group a hydrogen atom which can be shifted to the carbonyl oxygen atom and which may optionally be removed by dissociation in an alkaline medium. The type and size of the other substituents is not critical as long as the  $\alpha$ -aminocarbonyl compounds remain adequately soluble. The antioxidants according to the invention correspond in particular to the following general formula:



in which

10  $R^1, R^2, R^3$  and  $R^4$  are the same or different and represent hydrogen, hydrocarbon radicals including alkyl, cycloalkyl, for example cyclohexyl, or aryl, for example phenyl, which may also be further substituted, or heterocyclic groups, for example thienyl, with the proviso that the four radicals  $R^1, R^2, R^3$  and  $R^4$  do not simultaneously represent hydrogen.

15 In addition,

$R^1$  and  $R^2$  together may represent the radicals for completing a heterocyclic ring, for example a pyrrolidine, piperidine or morpholine ring, and/or

20  $R^2$  and  $R^3$  together may represent the radicals for completing a heterocyclic ring, for example a piperidine ring, and/or

25  $R^3$  and  $R^4$  together may represent the radicals for completing a heterocyclic or carbocyclic ring, preferably with 5, 6 or 7 ring members, more especially a carbocyclic ring, for example a cyclohexanone ring, and/or

30  $R^4$  and  $R^1$  together may represent the radicals for completing a heterocyclic ring, for example a piperidone ring.

35 An alkyl group represented by one of the radicals  $R^1, R^2, R^3$  and  $R^4$  preferably contains up to 5 carbon atoms, for example methyl, ethyl or butyl. These alkyl groups may contain further substituents, for example hydroxyl groups, amino groups or phenyl groups. Examples of particularly suitable substituted alkyl radicals are poly-hydroxy alkyl radicals of the type present, for example, in sugar molecules.

40 Antioxidants suitable for the purposes of the present invention correspond for example to the following general formula:



45 in which

$R^1$  and  $R^2$  together represent the radicals for completing a heterocyclic ring, for example a piperidine, pyrrolidine or morpholine ring; and

50  $R^3$  and  $R^4$  are the same or different and represent hydrogen, alkyl, for example methyl, ethyl or butyl, including substituted alkyl radicals, aryl, for example phenyl, or heterocyclic groups.

55 According to the invention, other suitable antioxidants correspond, for example, to the following general formula:



60 in which



colour developer baths in the usual concentrations, for example in concentrations of from 0.5 to 25 g per liter.

In addition, the colour developer compositions according to the invention may contain other standard additives in the usual quantities, such as substances with an alkaline effect, for example alkali metal hydroxide, alkali metal carbonate, alkali metal phosphate or alkali metal borate, also alkali metal sulphite, alkali metal sulphate, alkali metal bromide or alkali metal iodide; silver salt solvents, for example alkali metal thiosulphate or alkali metal thiocyanate and, optionally, viscosity-increasing agents, such as hydroxyalkyl cellulose or carboxyalkyl celluloses. Instead of alkali metal ions, for example sodium or potassium ions, ammonium ions may be present in the above-mentioned additives. Other standard additives are anti-lime agents, for example, alkali metal phosphate, and alkali metal or ammonium salts of polyaminopolycarboxylic acids, for example nitrilotriacetic acid, ethylene diamine tetraacetic acid or 1,3-diaminopropanol tetraacetic acid, also salts of hydroxyethyl diphosphonic acid of the type described, for example, in DT-OS No. 2,227,639 or DT-OS No. 2,246,610. In addition, the colour developer compositions may contain soluble competitive couplers, for example citrazinic acid, development accelerators, for example polyethylene oxide derivatives or, in the case of reversal colour developer compositions, fogging agents, for example boron hydride compounds or hydrazine derivatives.

The anti-oxidation effect of the antioxidants used in accordance with the invention is superior both to that of hydroxylamine and also to that of some of the compounds described in U.S. Pat. No. 3,615,503. This is reflected in the fact that, in the colour developer compositions, the concentration of colour developer compound decreases less rapidly in the presence of the compounds according to the invention than in the presence of hydroxylamine or, for example, dihydroxy acetone or dihydroxy maleic acid. It has also been found that the antioxidants according to the invention do not themselves take any significant part in the development process, as is known to occur with hydroxylamine and has occasionally been observed under certain conditions, especially in colour reversal processing. In reversal colour development with colour developer baths containing hydroxylamine as antioxidant, fluctuations are occasionally observed in the colour density developed in dependence upon the concentration of hydroxylamine in the bath. By contrast, it is possible in cases where the antioxidants according to the invention are used, for example in cases where compound 1 is used, readily to accept fairly small fluctuations in the concentration of antioxidant without this being reflected in considerable deviations in the colour densities developed.

The antioxidants according to the invention are suitable for use in photographic colour developer baths of all kinds, for example for colour developer baths for the colour development of colour-photographic negative materials or for reversal colour developer baths for the development of colour photographic reversal materials. The advantages of the antioxidants according to the invention are particularly conspicuous in photographic colour developer baths of the type which are used at elevated temperatures and which remain in service for prolonged periods during colour photographic processing.

### EXAMPLE 1

Compounds 1, 2 and 3 were used as antioxidants, in comparison with hydroxylamine sulphate and dihydroxy acetone (U.S. Pat. No. 3,615,503), in a conventional colour developer bath of the following composition (H<sub>2</sub>O to 1000 ml):

|                                          |      |
|------------------------------------------|------|
| Sodium hexametaphosphate                 | 2 g  |
| Trisodium phosphate                      | 20 g |
| Sodium sulphite sicc.                    | 2 g  |
| Antioxidant according to Table 1 below   | 1 g  |
| N,N-diethyl-p-phenylene diamine sulphate | 5 g  |
| Potassium bromide                        | 1 g  |
| pH-value (with NaOH)                     | 12.3 |

15

The developers (1 liter of each) were poured into flat dishes (150 cm<sup>2</sup> air surface) and exposed for 1 week to atmospheric oxidation. Thereafter, they were made up to exactly 1 liter with distilled water. The residual concentration of colour developer was then determined by titration with a Ce(IV) solution.

The percentage reduction in the concentration of colour developer by atmospheric oxidation is shown in Table 1.

Table 1

| Compound               | Percentage reduction in concentration of colour developer |
|------------------------|-----------------------------------------------------------|
| Hydroxylamine sulphate | -20                                                       |
| Dihydroxy acetone      | -17.1                                                     |
| 1                      | -15.4                                                     |
| 2                      | -15.4                                                     |
| 3                      | -15.8                                                     |

### EXAMPLE 2

The test arrangement was as described in Example 1. Compounds 1, 3, 4, 5 and 6 were compared with dihydroxy acetone; exposure time to atmospheric oxygen 2 weeks.

The results are set out in Table 2.

Table 2

| Compound          | Percentage reduction in concentration of colour developer |
|-------------------|-----------------------------------------------------------|
| Dihydroxy acetone | -35.8                                                     |
| 1                 | -28.3                                                     |
| 3                 | -34.6                                                     |
| 4                 | -35.0                                                     |
| 5                 | -34.4                                                     |
| 6                 | -31.6                                                     |

55

### EXAMPLE 3

Compound 5 was used as antioxidant in comparison with dihydroxy acetone in a colour developer bath of the following composition (per 1000 ml) for colour negative material:

|                                          |        |
|------------------------------------------|--------|
| Sodium hexametaphosphate                 | 2 g    |
| Sodium sulphite sicc.                    | 2 g    |
| N,N-diethyl-p-phenylene diamine sulphate | 2.75 g |
| Antioxidant                              | 1.2 g  |
| Potassium carbonate sicc.                | 75 g   |
| Potassium bromide                        | 2 g    |



UNITED STATES PATENT AND TRADEMARK OFFICE  
CERTIFICATE OF CORRECTION

PATENT NO. : 4, 155, 764

Page 1 of 2

DATED : May 22, 1979

INVENTOR(S) : Melzer et al.

It is certified that error appears in the above-identified patent and that said Letters Patent are hereby corrected as shown below:

Column 2, general formula 1, the broken line between R<sup>1</sup> and R<sup>4</sup> should not touch the O atom. The formula should read:



Column 8, Line 2, the phrase "composition per 1000 ml" is misplaced. It should appear as follows, above the line:

-- composition per 1000 ml: --

UNITED STATES PATENT AND TRADEMARK OFFICE  
CERTIFICATE OF CORRECTION

PATENT NO. : 4,155,764

Page 2 of 2

DATED : May 22, 1979

INVENTOR(S) : Melzer et al.

It is certified that error appears in the above-identified patent and that said Letters Patent are hereby corrected as shown below:

Column 8, claim 1, the broken line between R<sup>1</sup> and R<sup>4</sup> should not touch the O atom. The formula should read:



Signed and Sealed this  
Sixth Day of May 1980

[SEAL]

Attest:

SIDNEY A. DIAMOND

Attesting Officer

Commissioner of Patents and Trademarks